

## UNITED STATES PATENT OFFICE.

FRITZ GÜNTHER, OF LUDWIGSHAFEN-ON-THE-RHINE, GERMANY, ASSIGNOR TO THE BADISCHE ANILIN- & SODA-FABRIK, OF LUDWIGSHAFEN-ON-THE-RHINE, GERMANY, A CORPORATION OF GERMANY.

## DYEING CELLULOSE ESTERS.

No Drawing.

Application filed April 9, 1923. Serial No. 630,942.

To all whom it may concern: .

Be it known that I, FRITZ GÜNTHER, citizen of the German Empire, residing at Ludwigshafen-on-the-Rhine, Germany, have invented new and useful Improvements in Dyeing Cellulose Esters, of which the following is a specification.

This invention relates to a process for dyeing cellulose esters which, as is known, has hitherto encountered great difficulty substantially caused by the property possessed by cellulose acetate of having no affinity for direct or acid coloring matters.

According to the present invention the dyeing of cellulose esters can be satisfactorily effected by employing insoluble or difficultly soluble azo dyestuffs in the form of their water soluble bisulfite derivatives. With such derivatives the cellulose acetate can be dyed in various ways for example from an aqueous dye bath at a moderate or hot temperature and the dye bath may have a weakly acid condition. For example the bisulfite compound of the azo coloring matter aniline-azo-beta-naphthol has been ascribed the following formula:



(see Woroshtzow, Journal für praktische Chemie, Vol. 84, 1911, page 523; another theory is given by the same author in Journal of the Russian physico-chemical Society, Vol. 47, page 1669).

In order to illustrate the nature of this invention, the following example is given, 40 but the invention is not restricted to this example.

The dye bath may contain the bisulfite compound of the azo coloring matter aniline-azo-beta-naphthol and also a small addition of acetic acid in order to increase its stability which dye bath may be kept at from about 50 degrees to 60 degrees centigrade. The cellulose acetate is introduced in a well wetted condition into said dye bath whereupon the temperature of the bath is gradually raised to about 70 degrees to 75 degrees centigrade. The dyed material is rinsed with water and then shows a beautiful golden orange color. 55

Bisulfite compounds of other insoluble or difficultly soluble azo dyestuffs and other cellulose esters may be employed in an analogous way.

I claim:

1. The process of dyeing cellulose esters, characterized by employing bisulfite compounds of difficultly soluble or insoluble azo coloring matters.

2. The process of dyeing cellulose acetate 65 silk which consists in treating the silk in a dye bath containing a water soluble bisulfite compound of a difficultly soluble or insoluble azo coloring matter and in a weak acid condition. 70

In testimony whereof I have hereunto set my hand.

FRITZ GÜNTHER.

Witnesses:

W. W. SCHOTT,  
C. C. L. B. WYLES.